# EUROPEAN PATENT SPECIFICATION

(11) **EP 0 734 430 B1**
(45) Date of publication and mention of the grant of the patent: **23.06.2004**
(21) Application number: 95904049.4
(22) Date of filing: 14.10.1994
(51) Int. Cl.: C10L 3/00, C10L 1/18

(54) **Hydrocarbon torch gas**
Kohlenwasserstoffgas für Schweissbrenner
Gaz d'hydrocarbures pour chalumeau

(43) Date of publication of application: 02.10.1996
(73) Proprietor: EXCELLENE LIMITED, Port Vila (VU)
(72) Inventor: FRITZ, James, Edward, Port Townsend, WA 98368 (US)
(74) Representative: Crump, Julian Richard John
(86) International application number: PCT/US1994/011619
(87) International publication number: WO 1996/011998

(56) References cited:
- WO-A-94/01515
- DE-A- 2 455 727
- GB-A- 569 108
- US-A- 3 869 262
- US-A- 5 232 464
- US-A- 5 236 467
- DATABASE WPI Section Ch, Week 9540 Derwent Publications Ltd., London, GB; Class H06, AN 95-311792 XP002085604 & ZA 9 408 012 A (EXCELLENE LTD) , 26 July 1995

## Description

### Technical Field

The present invention relates to hydrocarbon gas for use in cutting and/or welding torches fortified by the addition of an additive or conditioner, particularly a double additive.

### Background Art

Various attempts have been made heretofore to improve gas used in cutting and/or welding torches by adding an additive or a double additive to them. These prior art gases have been composed of various hydrocarbons from methane to octane and some have included propane and butane. Harris U.S. patent No. 1,565,935, issued December 15, 1925, for example, fortified a wet casinghead gas composed of methane, ethane, propane, butane and hexane by the addition of ethyl ether [diethyl ether] [(C₂H₅)₂O or C₄H₁₀O] or methyl ether [dimethyl ether] [(CH₃)₂O]. Another patent that proposed to add ethyl ether, also called ethyl oxide, to a gas including propane or butane and propane is White U.S. patent No. 2,513,769, issued July 4, 1950.

British patent specification No. 813,981, published May 27, 1959 (Oxy-Ferrolene Limited) proposes to add to hydrocarbon gas an oxygen-containing compound such as isopropyl ether [diisopropyl ether,] [(CH₃)₂CH₂O or (C₃H₇)₂ or C₆H₁₄O], methyl isopropyl ether, methyl propyl ether [(CH₃)CH₂CH₂OCH₃ or C₄H₁₀O], normal propyl ether, ethanol [CH₃CH₂OH] and methanol [CH₃OH]. This British patent also suggests the incorporation of more than one compound but does not suggest any specific double compounds.

Seley U.S. patent No. 2,411,759, issued November 26, 1946, does suggest the use of double additives, namely, ethyl oxide [diethyl ether or ethyl ether] [(C₂H₅)₂O] and benzine [benzene] [C₆H₆]. White U.S. patent No. 2,951,750, issued September 6, 1960, refers to the prior double additives for torch gas of dimethyl ether [methyl ether] [(CH₃)₂O] and benzine [benzene] [C₆H₆] at column 1, lines 21 to 25, presumably as disclosed in the Seley patent, and then proposes the use of the double additive of propylene oxide [1,2-epoxy propane] [C₃H₆O] and dimethyl ether [(CH₃)₂O] at column 1, lines 55 to 62, instead of using benzine and dimethyl ether.

In addition, Kessler U.S. patent No. 3,591,355, issued July 6, 1971, proposed the addition of methanol [CH₃OH] to a gas containing propane or a double additive to torch gas composed of a liquid alkanol such as methanol and a mixture of alkanes such as pentane and isopentane. White U.S. patent No. 3,989,479, issued November 2, 1976, also proposed the addition of methanol and British patent specification No. 569,108, accepted May 4, 1945, proposed the addition of ammonia. This British patent also recommended increasing the amount of propane in producer gas, water gas, Mond gas and other commercially available gas mixtures in which methane predominated.

Medsker U.S. patent No. 2,908,599, issued October 13, 1959, stated that methyl borate and acetone had been used previously in a fuel for torch use citing U.S. patent No. 2,281,910. The Medsker patent proposed a mixture of methyl borate and hexane as an additive for a gaseous fuel. The Bialosky et al. patent No. 2,281,910, issued May 5, 1942, discloses a liquid flux containing methyl borate and a ketone, such as acetone [CH₃COCH₃] or methyl ethyl ketone [1,2-butanone] [CH₃CH₂COCH₃], to be subjected to a stream of acetylene, hydrogen or similar combustible gas for coating the work with boric acid or oxide.

German Offenlegungssehrift No. 24 55 727, published May 28, 1975, proposes a multitude of additions for fortifying hydrocarbons including higher mono-,di- and polyalcohols having 5 to 20 carbon atoms in each molecule. It is stated at page 12, line 24 that:

The preferred alcohols are the mono-, di- and polyalcohols of the C₅ to C₈ hydrocarbons which ... contain pentanols, hexanols, heptanols, octanols, pentenols, hexenols, heptenols and octenols.

Belgian patent No. PV 35 394A, issued January 13, 1967, discloses a method and device for obtaining a fuel mixture of homogeneous composition by spraying into a gaseous aliphatic hydrocarbon fuel such as propane alone or mixed with propylene a conditioning liquid composed of five classes of ingredients, namely:
(a) a component of fuel in liquid form which is the same as the base fuel
(b) a combustion activator which can be ethyl ether or a halogeno-ether, particularly a chloroether;
(c) a high calorific value liquid hydrocarbon for enhancing the evaporation of the activator and which is soluble in the activator, such as 2-methyl-butane having the formula CH₃CH₂CH(CH₃)₂ in an amount approximately equal to the amount of activator, i.e., between 1% and 12%, and preferably between 5% and 10% of the weight of the fuel used;
(d) a liquid oxidation catalyst, preferably selected from among the constituents of pyridine bases, particularly the alkylpyridines where the alkyl groups are of low molecular weight in an amount between 0.1% and 1% of the weight of fuel; and
(e) a hydrotrope which can be a terpenic . hydrocarbon, preferably being mixed with a phenylcarbinol or a carbinol alkyl ether, as well as with an aliphatic ester of carboxylic aromatic acid, preferably methyl salicylate.
This five-component conditioning liquid mixture is sprayed into the gaseous fuel at the moment that it is used, so that there will be no preferential vaporization of any of the constituents of the conditioning liquid.

Belgian patent of addition No. BE-A-697,274, issued June 30, 1967, which constitutes an addition to the principal patent No. PV 35 394, discloses the use of an alternative type of combustion activator in the five-component conditioning liquid of the main patent which is sprayed into the gaseous fuel.

Instead of using ethyl ether or a halogeno-ether as disclosed by the main patent for the activator component, the patent of addition uses as a combustion activator a hydrocarbon-oxygenated derivative, particularly an aliphatic hydrocarbon belonging to the group of esters, ketones and olefin oxides having the general formula CₙHₘOₚ where n is an integer between 2 and 6, m is an integer between 2 n -2 and 2 n +2, and p is equal to 1 or 2. The specific activators disclosed are:
acetone (C₃H₆O)
ethyl methyl ketone (C₄H₈O)
mesityl oxide [4-methyl-3-penten-2-one] (CH₃)₂C=CHCOCH₃ (C₆H₁₀O)
ethyl acetate (C₄H₈O₂)
ethylene oxide (C₂H₄O)
propylene oxide (C₃H₆O)
butylene oxide [1,2-epoxybutane] (C₄H₈O)

The principal torch gas used heretofore has been acetylene which is comparatively expensive, difficult to store and to transport, requires the use of almost pure oxygen with it and forms persistently adherent scoria when used for cutting ferrous metal.

Also, methyl ethyl ketone (MEK) has been used by itself heretofore as an additive for torch gas.
WO-A-9401515, published 20 January 1994, discloses the addition of a fortifying mixture of methyleythlketone plus C₄H₁₀O or C₄H₁₀O₂ group hydrocarbons to a propane hydrocarbon base gas. Activated carbon is also included in the mixture as a catalyst to make an azeotropic mixture. The resulting liquified fuel gas improves motor vehicle performance, lowers harmful emissions and can be used with underwater cutting equipment with as little as 95% oxygen.

A principal object of this invention is to provide a simple additive for fortifying hydrocarbon torch gas so as to have characteristics superior to those of acetylene, especially for cutting ferrous metal, and also for welding. Such object also includes providing fortified hydrocarbon having characteristics superior to those of hydrocarbon fortified only by the addition of methyl ethyl ketone.

A particular object is to provide a torch gas which will have high flame temperature and intense heating capability.

A further object is to provide torch gas that can be stored and transported easily and economically.

Another object is to provide a torch gas having a base gas which is readily available in almost the entire world, can be provided more economically and is easy to fortify for enhancing its attributes.

It is also an object to provide a torch gas enabling ferrous metal to be cut faster and cleaner.

Another object is to provide a gas that can be used by torches for cutting under water at considerable depths.

An additional object is to provide a gas that can be used for torch cutting more economically because it will combine effectively with oxygen containing a higher proportion of adulterating gases which cannot be used with acetylene.

The foregoing objects can be accomplished by utilizing liquefied petroleum gas fortified with methyl ethyl ketone and with lower pluraloxyhydrocarbons, namely dioxy- and trioxyhydrocarbons having two to four carbon atoms in each molecule or with a combination of additions from such pluraloxyhydrocarbons and/or selected lower monooxyhydrocarbons having three or four carbon atoms in each molecule.

According to one aspect of the invention therefore there is provided a hydrocarbon torch gas which is a mixture of a hydrocarbon base gas and an additive characterised in that said additive comprises at least one alcohol component selected from the group consisting of 1, 2-ethandiol, 1, 2-propandiol, glycerol, n-propyl alcohol, isopropyl alcohol and at least a second component selected from the group consisting of ethylene glycol dimethyl ether, ethyl acetate, methyl ethyl ketone and butyraldehyde.

The total additive may be in an amount 0.5%-13% by weight of the hydrocarbon base gas. Preferably, the amount of additive is within a range of 3% to 7% by weight of the hydrocarbon base gas.

Preferably, the hydrocarbon torch gas is maintained under pressure.

The hydrocarbon base gas may be Liquified Petroleum Gas (LPG).

Liquefied petroleum gas (LPG) is the preferred base gas for the fortified torch gas of the present invention because of its high butane and propane content. Both the n-butane and isobutane isomers of butane are usually present in LPG, but a substantial amount of butane may have been removed from LPG sold as fuel because of the demand from industry for butane derivatives, in which case the LPG is composed largely of propane. It is, however, desirable that there be a reasonable proportion of butane in the LPG, such as from 5% to 40%.

Alternatively, the base gas could be propane or butane alone or any mixture of these gases or propylene or other gaseous hydrocarbon.

The additive or conditioner used to fortify the base gas may be simply a combination of methyl ethyl ketone (MEK), otherwise known as 2-butanone, having the formula CH₃COCH₂CH₃ and a lower pluraloxydrocarbon. MEK is a liquid with a boiling point of 70.6 degrees C. and a specific gravity of 0.805 at 20 degrees C.

LPG must be stored under pressure to keep it in a liquid state, but relatively heavy pressurized storage tanks and handling equipment for LPG is commercially practical and customary.

Without being fortified, LPG mixed with oxygen is not very effective for torch cutting and welding, not nearly as effective as acetylene gas mixed with substantially pure oxygen, but by enriching the base LPG with an effective additive the flame temperature is considerably increased and the heating capability is greatly improved.

The amount of additive used will depend on the extent to which it is desired to improve the characteristics of the base gas, but the amount would be 3% to 10% of the base gas by weight. Where a combination of MEK and a lower pluraloxyhydrocarbon is used, preferably 3% to 5% of MEK and 2% or 3% of the lower pluraloxyhydrocarbon is appropriate as the sole additive.

The procedure for combining the additive with the LPG is simple. The fortifying liquid is simply mixed with the hydrocarbon in liquid form. The additive which is liquid at normal temperatures is supplied to the storage tank in which the LPG under liquefying pressure is to be stored or transported. It is quite practical to supply the additive to standard 210 litres (55-gallon) drums.

If more additive is supplied than about 6% of the base gas by weight, such additive should be supplied in conjunction with a catalyst, preferably activated carbon in the form of powder, granules or pellets to insure homogeneous mixing. The activated carbon is amorphous, preferably having been produced from coal or petroleum coke. Alternative catalysts that can be used are platinum, cupric oxide and granular silver carried by a suitable carrier.

The amount of activated carbon used is not critical, but it should be placed in the bottom of a storage container to facilitate mixing of the additive with the hydrocarbon base gas when it is supplied to the container under pressure. An amount of such catalyst between 1% and 5% of the weight of the additive would be satisfactory. The resulting liquid mixture of base gas and additive or conditioner will be azeotropic at normal temperatures so that the fortified torch gas evaporated from the fortified liquid mixture will be homogeneous when it is released from the storage container to the torch without the addition of other hydrocarbon gas or being supplied to other hydrocarbon gas.

In order to provide an effective cutting flame, it is necessary to supply to an acetylene torch oxygen that is in substantially pure form, such as at least 99% oxygen by volume. Satisfactory cutting temperatures can be provided by mixing with the fortified base gas of the present invention less pure oxygen such as oxygen having a purity of approximately 95%, the adulterant being nitrogen, carbon dioxide and other gas components of air. Even when oxygen having a purity as low as 90% is used, the flame temperature of base LPC of approximately 5,000 degrees P. (2,760 degrees C.) can be raised to approximately 5,800 degrees F. (3204.44 degrees C.) to 6,000 degrees F. (3315.56 degrees C.) by use of the base LPG fortified by additives according to the present invention. Such impure oxygen can be produced economically by compressing air to about 27579029 pascals (4,000 psi) chilling it to minus 360 degrees F. (minus 217.78 degrees C.) which liquefies the air and then allowing the temperature of the liquefied air to rise gradually while venting the container to release the nitrogen component of the liquefied air which vaporizes at minus 320 degrees F. (minus 195.56 degrees C.) leaving the oxygen in liquid form.

In other processes for producing impure oxygen, nitrogen of the air is removed by zeolite resulting in oxygen of 90% to 95% purity.

An advantage of using the fortified base gas of the present invention over acetylene for cutting ferrous metal is that a clean precise kerf is obtained. oxyacetylene cutting produces a hard scoria persistently adherent to the work which increases the heating required and usually must subsequently be chipped off the work. Utilization of the fortified torch gas of the present invention produces a soft friable scoria which is sloughed off the work and out of the kerf as the cutting progresses to leave a narrower clean kerf with virgin metal along opposite margins of the kerf.

A particular advantage which the fortified torch gas of the present invention has is that it can be used for flame cutting under water to a depth of 91.5 metres (300 feet). The use of the oxyacetylene torch is limited to 6.1 metres (20 feet) under water because at pressures to which it would be necessary to subject the gas to enable it to be dispensed to the cutting torch at greater depths the acetylene will explode. Consequently, the only alternative that has been available for cutting under water at depths greater than about 6.1 metres (20 feet) prior to use of MEK as an additive to hydrocarbon gas has been the use of a carbon arc, the action of which is slow and the use of which is dangerous.

While the use of MEK has been beneficial in expediting cutting of metal, the use of MEK enhanced by the addition of tert-butyl alcohol (TBA) has increased the cutting speed from 5% to 10%, and the use of MEK and methyl tetra-butyl ether (MTBE) in combination has increased the cutting speed to 20% to 25% faster than where MEK has been used alone as an additive and about 15% faster than the cutting speed where the MEK has been enhanced with TBA. Use of MEK in conjunction with a lower pluraloxyhydrocarbon is preferable.

Use of hydrocarbon gas such as LPG for soldering, brazing or light metal cutting is rendered more effective if the additive of the present invention is mixed with the gas. For such use it is preferable to use less additive than in the case of torch gas for cutting or welding thick metal. For soldering, brazing or light cutting, an amount of additive within the range of 2% to 5% by weight is adequate, and such an amount can be mixed sufficiently intimately with the hydrocarbon gas without the use of a catalyst.

As alternatives to the use of a combination of MEK and a lower pluraloxyhydrocarbon described above the additive of the present invention may be simply a single lower pluraloxyhydrocarbon, namely, a dioxy- or trioxyhydrocarbon having from 2 to 4 carbon atoms in the molecule and which may be an alcohol, an ether or an acetate. Particular examples of such pluraloxyhydrocarbons are specified in the tables below:

| Name | Formula | Formula Weight |
|---|---|---|
| Dihydric Alcohols (Diols) | | |
| 1,2-ethanediol | C₂H₆O₂ | Formula Weight 62 |
| HOCH₂CH₂OH, also called ethylene glycol | | |
| | | |
| 1,2-propanediol | C₃H₈O₂ | Formula Weight 76 |
| CH₃CH(OH)CH₂OH, also called propylene glycol | | |
| | | |
| 1,3 butanediol | C₄H₁₀O₂ | Formula Weight 90 |
| CH₃CH(OH)CH₂CH₂OH, also called 1,3 butylene glycol | | |

| Trihydric Alcohols | | |
|---|---|---|
| glycerol | C₃H₈O₃ | Formula Weight 92 |
| HOCH₂CH(OH)CH₂OH | | |
| | | |
| diethylene glycol | C₄H₁₀O₃ | Formula Weight 106 |
| HOCH₂CH₂OCH₂CH₂OH, also called bis (2-hydroxyethyl) ether | | |

| Dioxyethers | | |
|---|---|---|
| ethylene glycol monomethyl ether | C₃H₈O₂ | Formula Weight 76 |
| CH₃OCH₂CH₂OH, also called 2-methoxyethanol | | |
| | | |
| ethylene glycol monoethyl ether | C₄H₁₀O₂ | Formula Weight 90 |
| CH₃CH₂OCH₂CH₂OH, also called 2-ethoxyethanol | | |
| | | |
| ethylene glycol dimethyl ether | C₄H₁₀O₂ | Formula Weight 90 |
| CH₃OCH₂CH₂OCH₃, also called 1,2 dimethoxyethane | | |

| Acetates | | |
|---|---|---|
| ethyl acetate | C₄H₈O₂ | Formula Weight 88 |
| CH₃COOC₂H₅, also called acetic ester or acetic ether | | |

The effect of various monooxyhydrocarbons to enhance the combustion of torch gases when used alone is varied and unpredictable. The following lower monooxyhydrocarbons are reasonably beneficial in combination or in combination with pluraloxyhydrocarbon as enhancing additives without the use of other additive components. Such monooxyhydrocarbons will have three or four carbon atoms in a molecule.

| Name | Formula | Formula Weight |
|---|---|---|
| Monohydric Alcohols | | |
| n-propyl alcohol | C₃H₈O | Formula Weight 60 |
| CH₃CH₂CH₂OH, also called 1-propanol | | |
| | | |
| isopropyl alcohol | C₃H₈O | Formula Weight 60 |
| (CH₃)₂CHOH, also called 2-propanol | | |
| | | |
| n-butyl alcohol | C₄H₁₀O | Formula Weight 74 |
| CH₃CH₂CH₂CH₂OH, also called 1-butanol | | |
| | | |
| isobutyl alcohol | C₄H₁₀O Formula Weight 74 | |
| (CH₃)₂CHCH₂OH, also called 2-methyl-1-propanol | | |
| | | |
| sec butyl alcohol | C₄H₁₀O | Formula Weight 74 |
| CH₃CH₂CH(OH)CH₃, also called 2-butanol | | |

| Ketones | | |
|---|---|---|
| methyl ethyl ketone | C₄H₈O | Formula Weight 72 |
| CH₃COCH₂CH₃, also called 2-butanone | | |

| Aldehydes | | |
|---|---|---|
| propionaldehyde | C₃H₆O | Formula Weight 58 |
| CH₃CH₂CHO, also called 1-propanal | | |
| | | |
| butyraldehyde | C₄H₈O | Formula Weight 72 |
| CH₃CH₂CH₂CHO | | |

While a single one of the monooxyhydrocarbons listed above does not individually enhance LPG, butane or propane gas sufficiently to be comparable to acetylene for use in cutting or welding, the combination of two or three additives selected from the monooxyhydrocarbons specified above and the dioxyhydrocarbons and trioxyhydrocarbons will provide greater enhancement than any one of such chemicals alone.

Also, while it is practical to utilize a single pluraloxyhydrocarbon as an additive, better results are obtained by combining pluraloxyhydrocarbons with each other or with a monooxyhydrocarbon of a suitable type without using other components in the additive.

For example, while LPG enhanced with 3% by weight of the base gas of either 1,2 ethanediol or ethylene glycol monomethyl ether will enable a perfect cut of steel to be made as rapidly as by the use of acetylene, a cutting operation in which the base gas is enhanced with 3% by weight of each of such additives will enable an excellent cut to be made at a rate faster than could be obtained using acetylene.

Also, as good and almost as fast a cut can be obtained by using as an additive 3% by weight of the base gas of 1,2-ethanediol and 2% by weight of the base gas of methyl ethyl ketone. Comparable results can be obtained by using 3% by weight of the base gas of ethylene glycol monomethyl ether and n-propyl alcohol.

While mention has been made of using 2% or 3% of each of two oxyhydrocarbons specified above in combination, it is also possible to obtain good enhancement by using a combination of 2% by weight of the base gas of each of three of the oxyhydrocarbons specified above.

## Claims

1. A hydrocarbon torch gas which is a mixture of a hydrocarbon base gas and an additive **characterised in that** said additive comprises at least one alcohol component selected from the group consisting of 1,2-ethandiol, 1, 2-propandiol, glycerol, n-propyl alcohol, isopropyl alcohol and at least a second component selected from the group consisting of ethylene glycol dimethyl ether, ethyl acetate, methyl ethyl ketone and butyraldehyde.

2. A hydrocarbon torch gas as claimed in claim 1, wherein the total additive is in an amount 0.5%-13% by weight of the hydrocarbon base gas.

3. A hydrocarbon torch gas as claimed in claim 1 or claim 2, wherein said hydrocarbon base gas is Liquified Petroleum Gas.

## Patentansprüche

1. Kohlenwasserstoffgas für Brenner, das ein Gemisch aus einem Kohlenwasserstoffbasisgas und einem Zusatz ist, **dadurch gekennzeichnet, dass** der Zusatz mindestens eine Alkoholkomponente, die aus der Gruppe bestehend aus 1,2-Ethandiol, 1,2-Propandiol, Glycerol, n-Propylalkohol, Isopropylalkohol ausgewählt ist, und mindestens eine zweite Komponente enthält, die aus der Gruppe bestehend aus Ethylenglykoldimethyläther, Ethylacetat, Methylethylketon und Butyraldehyd ausgewählt ist.

2. Kohlenwasserstoffgas für Brenner nach Anspruch 1, wobei die Gesamtmenge des Zusatzes 0,5-13 Gew.-% des Kohlenwasserstoffbasisgases beträgt.

3. Kohlenwasserstoffgas für Brenner nach Anspruch 1 oder 2, wobei das Kohlenwasserstoffbasisgas verflüssigtes Erdölgas ist.

## Revendications

1. Gaz hydrocarbure pour chalumeau qui est un mélange d'un gaz de base hydrocarbure et d'un additif **caractérisé en ce que** ledit additif comprend au moins un composant alcool choisi dans le groupe constitué par le 1,2-éthanediol, le 1,2-propanediol, le glycérol, l'alcool n-propylique, l'alcool isopropylique et au moins un second composant choisi dans le groupe constitué par le diméthyléther d'éthylène glycol, l'acétate d'éthyle, la méthyléthylcétone et le butyraldéhyde.

2. Gaz hydrocarbure pour chalumeau selon la revendication 1, dans lequel l'additif total est dans une quantité de 0,5 % à 13 % en poids des gaz de base hydrocarbures.

3. Gaz hydrocarbure pour chalumeau selon la revendication 1 ou 2, dans lequel le gaz de base hydrocarbure est du gaz de pétrole liquéfié (GPL).
